

July 26, 1949.

C. C. PATTON

2,477,139

CONDUCTING BEARING

Filed April 4, 1944



INVENTOR.  
C. C. PATTON  
BY  
*Harry L. Dingle*  
ATTORNEY

Patented July 26, 1949

2,477,139

# UNITED STATES PATENT OFFICE

2,477,139

## CONDUCTING BEARING

Charles C. Patton, Chicago, Ill., assignor to Western Electric Company, Incorporated, New York, N. Y., a corporation of New York

Application April 4, 1944, Serial No. 529,516

4 Claims. (Cl. 308—237)

1

This invention relates to conducting bearings and more particularly to a friction bearing having a high degree of electrical conductivity between the frictionally moving elements thereof.

It is an object of the present invention to provide a bearing having a high degree of electrical conductivity and a low degree of friction between its elements and a method of producing such a bearing.

In accordance with one embodiment of the invention as applied to bearings adapted to electrically interconnect two elements and at the same time provide as frictionless a contact as possible between the elements, the bearing surface of one of the relatively rotatable elements is provided with a gold plating and the other of the bearing surfaces is gold plated on copper, which, in turn, is applied on a base metal and wherein the copper-gold-base metal is heat-treated to effect a partial alloying of the copper and gold, thereby to present a hard gold surface for engagement with the soft gold surface on the other bearing element.

A complete understanding of the invention may be had by reference to the following detailed description when considered in conjunction with the accompanying drawing, wherein

Fig. 1 is a side elevational view on a greatly enlarged scale, partly in section, of a pair of bearing members mounted in telescoping relation and having bearing surfaces formed in accordance with the present invention and

Fig. 2 is a sectional view taken substantially along the line 2—2 of Fig. 1 in the direction of the arrows.

In some forms of electrical apparatus, notably radio apparatus, it is sometimes desirable to electrically interconnect two members which must move relative one to the other, and to protect said surfaces from deleterious oxidation and corrosion. In the present embodiment of the invention, these two members have been shown as two tubular relatively rotatable elements, designated generally by the numerals 3 and 4. In order to increase the degree of conductivity between the two members 3 and 4, which may comprise bases 5 and 6, respectively, made of brass and steel, the brass surface may be plated with a metal of high conductivity, such as gold, which is applied thereto in a thin coating 7. The outer surface of the element 6, which is to bear in and be electrically conductive with respect to the element 3, has, in accordance with the present invention, a plating 8 of copper applied thereto by any suitable method, for ex-

2

ample, by electroplating it and, thereafter, the copper plate 8 has a plating 9 of gold applied to it to bear against the plating 7 of gold on the brass tube 5. The gold plated surface 7 of the element 3 may be used in the same condition that it attains when it is plated thereon. In other words, the plating 7 of gold will be relatively soft. However, in order to prevent the plating 9 of gold on the inner element 4 from seizing when the elements 3 and 4 are moved relative one to another, the element 3, with the plating 8 of copper and 9 of gold thereon, is heat-treated to effect an interalloying or penetration of copper into the gold and the gold into the copper, thus to harden the outer surface of the gold.

In the preferred embodiment of the invention, the steel tube, after it has been properly machined, may be plated with approximately .005" of copper and upon the copper there may be plated .002" of gold. After the copper and gold in superposed relation have been plated onto the steel tube 6, the tube is heat-treated at 800° F. for approximately one-half hour and, when so treated, there will be a penetration or alloying of the copper into the gold and the gold into the copper. As viewed under a microscope, the penetration of the copper into the gold and the gold into the copper is quite irregular and apparently a complete alloying of the two metals does not take place, but some of the hardening characteristics of the copper seem to extend to the outer surface of the gold so that, with respect to the plain gold-plated brass tube 3, the bearing surface on the tube or element 4 is quite hard and when the two elements are moved with respect one to another, the friction between them is quite low. The migration or diffusion of the gold into the copper and copper into the gold during the heat treatment sometimes results in the formation of a visible copper scale on the outer surface of the gold, indicating that some of the copper travels completely through the plating of gold. When this occurs, the copper scale may be removed by dipping the bearing in a mild solution of nitric acid. In this manner, a friction bearing is provided which has substantially the same conductivity across its bearing surface as would be provided by two soft gold surfaces in engagement with one another, but has none of the tendency of two soft gold surfaces to grab or seize when they are moved with respect to another.

What is claimed is:

55 1. A frictional bearing comprising a metal

foundation having a copper surface, a gold plated coating over the copper surface and interalloyed therewith, and a frictional member having a base metal foundation provided with a gold plated friction surface.

2. In an electrically conductive corrosion resistant low friction bearing, a bearing member having a pure gold bearing surface, and a bearing member having a surface coating in engagement with the pure gold bearing surface, said 10 surface coating being harder than said pure gold bearing surface and comprising a layer of copper and a layer of gold superposed on said layer of copper and interdiffused therewith.

3. In an electrically conductive corrosion resistant low friction bearing, a bearing member having a gold bearing surface, and a bearing member comprising a hard base metal, a layer 15 of copper on the base metal, and a layer of gold on and interpenetrated with the layer of copper.

4. In an electrically conductive corrosion resistant low friction bearing, a bearing member having a pure gold bearing surface, and a bearing member comprising a relatively hard base 20 metal, a layer of copper plated on said base metal,

and a layer of gold plated on and partially interalloyed with said layer of copper.

CHARLES C. PATTON.

#### REFERENCES CITED

The following references are of record in the file of this patent:

#### UNITED STATES PATENTS

| Number    | Name        | Date           |
|-----------|-------------|----------------|
| 376,900   | Morell      | Jan. 24, 1888  |
| 1,600,961 | Payne       | Sept. 21, 1926 |
| 1,823,450 | Helmond     | Sept. 15, 1931 |
| 2,145,460 | Ryder       | Jan. 31, 1939  |
| 2,203,411 | Green       | June 4, 1940   |
| 2,241,739 | Queneau     | May 13, 1941   |
| 2,266,320 | Hobbs       | Dec. 16, 1941  |
| 2,283,219 | McCullough  | May 19, 1942   |
| 2,297,385 | Bierdermann | Sept. 29, 1942 |
| 2,316,119 | Bagley      | Apr. 6, 1943   |

#### FOREIGN PATENTS

| Number  | Country       | Date          |
|---------|---------------|---------------|
| 441,812 | Great Britain | Jan. 27, 1936 |